

Sept. 14, 1937.

H. RENCK

2,093,098

METHOD FOR PRODUCING CHEMICALS, ESPECIALLY AMALGAMATED PRINTING PLATES

Filed Sept. 25, 1935

*Fig. 1*



*Fig. 2*



*Fig. 3*



*Inventor:*

HEINRICH RENCK

By *Heinrich Renck*

*Attorney.*

## UNITED STATES PATENT OFFICE

2,093,098

METHOD FOR PRODUCING CHEMICALS,  
ESPECIALLY AMALGAMATED PRINTING  
PLATES

Heinrich Renck, Hamburg, Germany

Application September 25, 1935, Serial No. 42,059  
In Germany May 15, 1935

2 Claims. (Cl. 41—41.5)

The invention consists in an improvement of the well-known processes for producing ink-repellent portions on a printing plate. The known processes employ metallic mercury mixture, preferably glycerine to which metallic mercury is added. The mercury separating from the glycerine forms on the portions of the printing plate which must be ink-repellent a soft layer of mercury, i. e. a soft amalgam which, during the printing, is very soon squeezed out so that only a very limited number of prints can be made.

The invention has for its object to form a solid amalgam layer on the ink-repellent portions of the printing plate and with this object in view the glycerine is saturated with a mixture of ground nitrate of silver and ground nitrate of mercury.

These mixtures are added in the following proportions:—To 2 litres of glycerine 10 grams of ground nitrate of silver and 100 grams of nitrate of mercury are added.

The preparation is applied on to the denickeled portions of the printing plate so that the nitrate of silver and the nitrate of mercury deposit on these portions and form on the same a solid amalgam layer which has an ink-repellent effect during the printing.

A printing plate is produced in the following manner by the process according to the invention:

A brass coated iron plate is nickel-plated and the printing or design to be reproduced is transferred on to this nickel surface. The nickel is then removed from the portions which are not

covered by the transfer. The process up to this point does not differ from the known processes.

According to the invention nitrate of silver and nitrate of mercury are rubbed to a powder and dissolved in glycerine to saturation, whereupon this saturated glycerine is applied on the denickeled portions of the plate and here forms a solid amalgam layer.

The accompanying drawing shows the plate in the three different stages of its production.

Fig. 1 shows the iron plate 1 with the brass coating 2 and the nickel coating 3 with the transfer 4 applied thereon.

Fig. 2 shows the plate after the removal of the nickel coating 3 at the portions not covered by the transfer 4.

Fig. 3 shows the plate with solid amalgam layer 5 in the denickeled portions of the plate.

I claim:

1. Method of producing an ink repellent amalgam layer on certain portions of a printing plate, consisting in nickel-plating an iron plate coated with brass, applying the picture on the nickel-plated surface, removing the nickel-plating at the portions not covered by the picture, grinding together to a powder nitrate of silver and nitrate of mercury, dissolving this mixture in glycerine to saturation and applying this saturated solution on the denickeled portions of the plate.

2. In a method as specified in claim 1, in which the saturated glycerine solution consists of 10 grams of nitrate of silver and 100 grams of nitrate of mercury dissolved in 2 litres of glycerine.

HEINRICH RENCK.